

## UNITED STATES PATENT OFFICE

2,313,498

## CYANOACETYL COUPLER

Charles F. H. Allen and Paul W. Vittum, Rochester, N. Y., assignors to Eastman Kodak Company, Rochester, N. Y., a corporation of New Jersey

No Drawing. Application December 23, 1940, Serial No. 371,396. In Great Britain January 2, 1940

21 Claims. (Cl. 95—6)

This invention relates to photography and more particularly to compounds which form dyes by coupling with the developing compound on development.

The method of forming colored photographic images by depositing a colored compound in the photographic layer adjacent to the silver image has been described in numerous prior patents. The present invention relates to a process in which the color-forming compound is contained preferably in the developing solution, but might also be in the sensitive material, and forms a dye concurrently in the region adjacent to silver formed on development of the silver image by coupling with the oxidation product of the photographic developer. In U. S. Patent No. 2,115,394, granted April 26, 1938, to Mannes, Godowsky and Peterson, there are disclosed cyanoacetyl compounds useful as coupler compounds in photographic developers. In U. S. Patents Nos. 2,113,330, granted April 5, 1938, to Mannes and Godowsky, and 2,108,602, granted February 15, 1938, to Mannes and Godowsky, other cyanoacetyl compounds are disclosed.

We have found that there are certain cyanoacetyl coupler compounds which have better photographic characteristics than those which have hitherto been known. These new cyanoacetyl couplers which we describe have sharper absorption bands and considerably higher transmissions in a region of the spectrum such as the blue, with the result that satisfactory colors for subtractive color processes are obtained upon coupler development.

The compounds which we contemplate using have the general formula:



Where X is a CN or COOR<sub>3</sub> group, R<sub>3</sub> is alkyl, Z is NHR<sub>1</sub> or alkoxy, R<sub>1</sub> and R<sub>2</sub> are H, alkyl or aryl, Y is oxygen, sulfur or NR<sub>4</sub>, where R<sub>4</sub> is H, alkyl, or aryl.

Compounds which fall under this general classification are:

- (1) NH<sub>2</sub>—CO—NH—CO—CH<sub>2</sub>—CN  
Cyanoacetyl urea
- (2) NH<sub>2</sub>—CO—NH—CO—CH<sub>2</sub>—COOC<sub>2</sub>H<sub>5</sub>  
Ethyl malonyl urea
- (3) NH<sub>2</sub>—C—NH—CO—CH<sub>2</sub>—CN  
||  
NH  
Cyanoacetyl guanidine
- (4) CH<sub>3</sub>  
||  
NH—CO—NH—CO—CH<sub>2</sub>—CN  
Butyl cyanoacetyl urea

|     |                                                                                               |
|-----|-----------------------------------------------------------------------------------------------|
| (5) | C <sub>6</sub> H <sub>5</sub><br>NH—CO—NH—CO—CH <sub>2</sub> —CN<br>Phenyl cyanoacetyl urea   |
| (6) | C <sub>12</sub> H <sub>25</sub><br>NH—CO—NH—CO—CH <sub>2</sub> —CN<br>Lauryl cyanoacetyl urea |
| (7) | NH <sub>2</sub> —CS—NH—CO—CH <sub>2</sub> —CN<br>Cyanoacetyl thiourea                         |
| (8) | NC—NH—CO—CH <sub>2</sub> —CN<br>Cyanoacetyl cyanamide                                         |
| (9) | C <sub>2</sub> H <sub>5</sub> O—CO—NH—CO—CH <sub>2</sub> —CN<br>Cyanoacetyl urethane          |

These compounds, according to their molecular size and solubility, may be incorporated either in photographic emulsions or in developing solutions. Usually the less highly N-substituted compounds (those compounds having substituents of lower molecular weight) are used in developers. Compounds 1—5 and 7—9 are suitable for use in a developing solution and compound 6 may be incorporated into an emulsion layer. These couplers must contain a coupling function, which is in this case a reactive methylene group. By "coupling function" we mean a functional or reactive group common to coupler compounds which react with primary aromatic amino developers. By "reactive methylene" we mean a CH<sub>2</sub> group which is reactive in the coupling process. The reactive methylene group is present between two negative centers as in the groups —CO—CH<sub>2</sub>—CO— or —CO—CH<sub>2</sub>—CN. One of the atoms of the methylene group may, in general be substituted without destroying the chemical activity of the group, if the substituent is one which is split off easily such as halogen or carboxyl.

The aromatic amino developing agents used with the coupler compounds of our invention include the mono-, di-, and tri-aminoaryl compounds and their derivatives formed by substitution in the amino group as well as in the ring, such as alkylphenylenediamines and alkyltoluenediamines. These compounds are usually used in the salt form, such as the hydrochloride or the sulfate, which are more stable than the amines themselves. Suitable compounds are diethyl-p-phenylenediamine hydrochloride, mono-methyl-p-phenylenediamine hydrochloride, di-methyl-p-phenylenediamine hydrochloride and dimethyl-p-phenylenediamine sulfate. The p-aminophenols and their substitution products may also be used where the amino group is unsubstituted. All of these compounds have an unsubstituted amino group which enables oxida-

tion products of the developer to couple with the color forming compounds to form a dye image.

The following developer formula may be used with the compounds of our invention:

|                                        |       |     |
|----------------------------------------|-------|-----|
| A. p-Aminodiethyl aniline sulfate      | grams | 2   |
| Sodium sulfite anhydrous               | do    | 5   |
| Sodium carbonate anhydrous             | do    | 20  |
| Potassium bromide                      | do    | 2   |
| Water to                               | liter | 1   |
| <br>B. Coupler                         | grams | 1-5 |
| Solvent (acetone or isopropyl alcohol) | cc    | 100 |

Add B to A.

Our development process may be employed for the production of colored photographic images in layers of gelatin or other carrier such as collodion, organic esters of cellulose or synthetic resins. The support for the emulsion may be a transparent material such as glass, a cellulose ester, or an opaque material such as paper or an opaque cellulose ester. The superimposed layers may be sensitized to record different regions of the spectrum.

The cyanoacetyl couplers which we use are, in general, prepared by the interaction of cyanoacetic acid and ureas, guanidines, cyanamide or urethane in the presence of a dehydrating agent such as phosphorous oxychloride or acetic anhydride in a manner similar to that described in the German Patents Nos. 175,415 and 115,253. The malonyl urea couplers are prepared by the interaction of an acid chloride of malonic ester and a urea, thiourea, guanidine, etc. as described in the German Patent No. 193,447.

The methods and compounds set forth in the present specification are illustrative only and it is to be understood that our invention is limited only by the scope of the appended claims.

We claim:

1. A color forming photographic developer comprising an aromatic amino developing compound containing a primary amino group and a coupler compound having the formula:



where X is selected from the group consisting of CN and COOR<sub>3</sub> where R<sub>3</sub> is alkyl, Z is selected from the group consisting of NHR<sub>1</sub> and alkoxy R<sub>1</sub> and R<sub>2</sub> are selected from the group consisting of H, alkyl and aryl, Y is selected from the group consisting of oxygen, sulfur and NR<sub>4</sub>, where R<sub>4</sub> is selected from the group consisting of H, alkyl and aryl.

2. A color forming photographic developer comprising an aromatic amino developing compound containing a primary amino group and a coupler compound having the formula:



where R<sub>1</sub>, R<sub>2</sub>, and R<sub>4</sub> are selected from the group consisting of H, alkyl and aryl.

3. A color forming photographic developer comprising an aromatic amino developing compound containing a primary amino group and cyanoacetyl guanidine.

4. A color forming photographic developer comprising an aromatic amino developing compound containing a primary amino group and a coupler compound having the formula:



where R is alkyl, and R<sub>1</sub> and R<sub>2</sub> are selected from the group consisting of H, alkyl and aryl, Y is selected from the group consisting of oxygen, sulfur and NR<sub>4</sub>, where R<sub>4</sub> is selected from the group consisting of H, alkyl and aryl.

5. A color forming photographic developer comprising an aromatic amino developing compound containing a primary amino group and ethyl malonyl urea.

6. A color forming photographic developer comprising an aromatic amino developing agent containing a primary amino group and a coupler compound having the formula:



where R<sub>1</sub> and R<sub>2</sub> are selected from the group consisting of H, alkyl and aryl, Y is selected from the group consisting of oxygen and sulfur.

7. A color forming photographic developer comprising an aromatic amino developing compound containing a primary amino group and cyanoacetyl urea.

8. The method of producing a colored photographic image in a light sensitive silver halide emulsion layer which comprises exposing the layer and developing it with an aromatic amino developing compound containing a primary amino group in the presence of a coupler compound having the formula:



where X is selected from the group consisting of CN and COOR<sub>3</sub> where R<sub>3</sub> is alkyl, Z is selected from the group consisting of NHR<sub>1</sub> and alkoxy R<sub>1</sub> and R<sub>2</sub> are selected from the group consisting of H, alkyl and aryl, Y is selected from the group consisting of oxygen, sulfur and NR<sub>4</sub> where R<sub>4</sub> is selected from the group consisting of H, alkyl and aryl.

9. The method of producing a colored photographic image in a light sensitive silver halide emulsion layer which comprises exposing the layer and developing it with an aromatic amino developing compound containing a primary amino group in the presence of a coupler compound having the formula:



where R<sub>1</sub>, R<sub>2</sub> and R<sub>4</sub> are selected from the group consisting of H, alkyl and aryl.

10. The method of producing a colored photographic image in a light sensitive silver halide emulsion layer which comprises exposing the layer and developing it with an aromatic amino developing compound containing a primary amino group in the presence of cyanoacetyl guanidine.

11. The method of producing a colored photographic image in a light sensitive silver halide emulsion layer which comprises exposing the layer and developing it with an aromatic amino developing compound containing a primary amino group in the presence of a coupler compound having the formula:



where R is alkyl, and R<sub>1</sub> and R<sub>2</sub> are selected from the group consisting of H, alkyl and aryl, Y is selected from the group consisting of oxygen, sulfur and NR<sub>4</sub>, where R<sub>4</sub> is selected from the group consisting of H, alkyl and aryl.

12. The method of producing a colored photographic image in a light sensitive silver halide emulsion layer which comprises exposing the layer and developing it with an aromatic amino developing compound containing a primary amino group in the presence of ethyl malonyl urea.

13. The method of producing a colored photographic image in a light sensitive silver halide emulsion layer which comprises exposing the layer and developing it with an aromatic amino developing compound containing a primary amino group in the presence of a coupler compound having the formula:



where  $R_1$  and  $R_2$  are selected from the group consisting of H, alkyl and aryl, Y is selected from the group consisting of oxygen and sulfur.

14. The method of producing a colored photographic image in a light sensitive silver halide emulsion layer which comprises exposing the layer and developing it with an aromatic amino developing compound containing a primary amino group in the presence of cyanoacetyl urea.

15. A photographic emulsion for forming colored images comprising a carrier containing a sensitive silver halide and a coupler compound having the formula:



where X is selected from the group consisting of CN and  $COOR_3$  where  $R_3$  is alkyl, Z is selected from the group consisting of  $NHR_1$  and alkoxy  $R_1$  and  $R_2$  are selected from the group consisting of H, alkyl and aryl, Y is selected from the group consisting of oxygen, sulfur and  $NR_4$  where  $R_4$  is selected from the group consisting of H, alkyl and aryl.

16. A photographic emulsion for forming colored images comprising a gelatino silver halide

emulsion having incorporated therein a coupler compound having the formula:



5 where  $R_1$ ,  $R_2$ , and  $R_4$  are selected from the group consisting of H, alkyl and aryl,  $R_4$  is selected from the group consisting of H, alkyl and aryl.

17. A photographic emulsion for forming colored images comprising a gelatino silver halide emulsion having incorporated therein cyanoacetyl guanidine.

18. A photographic emulsion for forming colored images comprising a gelatino silver halide emulsion having incorporated therein a coupler compound having the formula:



20 where R is alkyl, and  $R_1$  and  $R_2$  are selected from the group consisting of H, alkyl and aryl, Y is selected from the group consisting of oxygen, sulfur and  $NR_4$ , where  $R_4$  is selected from the group consisting of H, alkyl and aryl.

19. A photographic emulsion for forming colored images comprising a gelatino silver halide emulsion having incorporated therein ethyl malonyl urea.

20. A photographic emulsion for forming colored images comprising a gelatino silver halide emulsion having incorporated therein a coupler compound having the formula:



35 where  $R_1$  and  $R_2$  are selected from the group consisting of H, alkyl and aryl, Y is selected from the group consisting of oxygen and sulfur.

21. A photographic emulsion for forming colored images comprising a gelatino silver halide emulsion having incorporated therein cyanoacetyl urea.

CHARLES F. H. ALLEN.  
PAUL W. VITTM.